

Nov. 24, 1936.

W. HESSENBRUCH

2,062,130

HEAT TREATABLE NICKEL-BERYLLIUM ALLOYS

Filed March 23, 1935

Fig. 1.



Fig. 2.



Fig. 3.



Werner Hessenbruch  
BY  
Symmetzky & Lechner  
ATTORNEYS

## UNITED STATES PATENT OFFICE

2,062,130

HEAT TREATABLE NICKEL-BERYLLIUM  
ALLOYS

Werner Hessenbruch, Hanau-on-the-Main, Germany, assignor to Heraens-Vacuumschmelze, A. G., Hanau-on-the-Main, Germany

Application March 23, 1935, Serial No. 12,586  
In Germany March 24, 1934

3 Claims. (Cl. 75—170)

This invention relates to nickel-beryllium alloys for springs and the like. It is known that nickel-beryllium alloys have been produced with a beryllium content of about 2½%, which permits improvement in hardness and in mechanical properties by heat treatment of about 1000° C., following quenching and reheating between 300—500° C. Similar to copper-beryllium alloys, nickel-beryllium alloys have found use for the manufacture of various springs. It has been found to be particularly difficult to obtain a maximum of hardness for thin springs or thin needles of beryllium-nickel alloys. The reason for this is the fact that it is very difficult to heat treat these small sections and the danger of over heat treatment exists, i. e., that the material gets soft again.

It has been found now that a greater persistency of the maximum hardness produced by heat treatment can be obtained if one part of the beryllium content is replaced by other elements, or that other elements are added to the alloy. It is known that with additions of any kind to a heat treatable alloy the limit of solubility of the mixed crystal containing beryllium can be shifted upward or downward. It has not been known, however, so far, that through such additions the stability of the maximum hardness produced by heat treatment of beryllium-nickel alloys can be greatly increased, and that the danger of softening by over heat treating can be reduced.

Careful experiments have shown that such elements have produced such greater stability through heat treatment which formed such heat treatable alloys with nickel, though a number of other elements will act in the same way though they, themselves, will not form heat treatable alloys with nickel.

In this case special additions of titanium has been found to be very useful. Through combination of this element with beryllium-nickel alloys it is possible to obtain results which far exceed the effect of the beryllium and the other additions alone. For instance, these conditions exist with respect to a nickel-titanium-beryllium alloy. Figure 1 shows the hardness of an alloy of nickel with 1% beryllium after quenching from about 1000° C. in water and annealing at various temperatures. As one sees from the curve, nickel-beryllium alloys, with 1% beryllium, show hardly any effect to heat treatment by annealing and

quenching. Figure 2 shows the Brinell hardness of a 3% titanium alloy as dependent on the annealing temperature after quenching from 1000° C. It is demonstrated here that by the titanium content a subsequent hardening by segregation has been obtained, but that at higher temperatures a quick softening will take place.

However, as shown in Figure 3, the heat treatment curve of an alloy with 3% titanium and 1% beryllium clearly shows that a very considerable increase in hardness can be obtained by quenching, followed by annealing at about 400—500° C., which greatly surpasses the hardness of both binary alloys and which remains intact even if the alloys are annealed for many hours.

These alloys have, in addition to their greater constancy, the advantage that low beryllium content produces strong and stable heat treatment effects, so that the use of these alloys in contradistinction to binary nickel-beryllium-alloys constitutes technical progress. This is true especially for all cases where these alloys are used for springs, for spring parts, or appliances, or for springy needles of all kinds.

In case a resistance against corrosion or against the effect of higher temperatures exceeding the natural properties of these alloys is needed, then to such alloys can be added chromium in quantities of substantially above a trace (about 0.5%) to about 30%. When using titanium, the intended effect can be obtained by additions from about .5% up to 10%.

I claim:

1. A nickel base alloy containing beryllium from a substantial amount above a trace to less than 2.5%, and titanium from about .5% to about 10%, said alloy being characterized by capacity to harden by heat treatment to increasing degrees of hardness in accordance with the temperature of heat treatment, and further being characterized by capacity to maintain hardness imparted by heat treatment even when heat treated for an extended period of time.

2. An alloy composed of 1% beryllium, 3% titanium and the balance nickel.

3. An alloy composed of beryllium from a substantial amount above a trace to less than 2.5%, and titanium from about .5% to about 10%, and the balance nickel.

WERNER HESSENBRUCH. 50